

## UNITED STATES PATENT OFFICE.

ERNST G. HONES, OF DUSSELDORF, GERMANY.

## TOOL FOR GUIDING AND SHAPING METAL AND THE LIKE.

No Drawing.

Application filed June 29, 1925. Serial No. 40,454.

*To all whom it may concern:*

Be it known that I, ERNST G. HONES, a citizen of Germany, residing at Dusseldorf, Bleichstr. 16/18, Germany, have invented 5 certain new and useful Improvements in Tools for Guiding and Shaping Metal and the like, of which the following is a specification.

This invention relates to tools for guiding 10 and shaping metal or the like, particularly in rolling processes or mills.

The tools which are used for guiding and shaping metal in rolling processes or mills are necessarily subjected to an extraordinary 15 amount of wear and tear. This applies particularly to piercing tools or mandrels of tube rolling mills, guide bars, direction changing members and such other tools as are employed in hot metal work, where they 20 are directly exposed and subjected to the action of heated metal.

Among the materials that were first used 25 for tools of this kind, was hard cast metal which, however, was soon found to have very small powers of resistance. Steel alloys such as chrome alloys etc., were then used for such tools and this material was found to be more satisfactory and superior to the hard cast metal, but even these tools are 30 quickly worn out and give rise to much annoyance in practice, as they must frequently be replaced etc. Furthermore, the irregular wear due to the irregular stresses on the tools frequently impairs the product obtained by them.

The object of this invention is to overcome these drawbacks. To this end it has 35 been found by exhaustive experiments, that a tool consisting of a steel alloy with additions of copper (Cu), zirconium (Z) and

cobalt (Co) amounting to from 0.1 up to 3 per cent has extraordinarily increased resistive powers.

In addition to the said substances, the alloy may contain admixtures of materials 45 that improve the quality of the tool material, such for instance as nickel, chrome, tungsten etc. It has been found that a tool consisting of such an alloy, and which can be formed into the desired shape by casting 50 for example, has a very much longer life than the tools made of materials hitherto employed. The resistive power of parts and tools which are subjected to hot material in a rolling process, as for example, the piercing tools or mandrels employed in producing seamless tubes or the guide members in rolling mills, amounts to several times that of the best steel tools produced by previous processes.

This novel material has also been found to be highly suitable for tools for guiding and shaping material or metal that is rolled or drawn in a cold state.

I claim:

1. A tool of the character described, composed of a steel alloy containing admixtures of copper, from 0.1 to 3 per cent; zirconium from 0.1 to 3 per cent; and cobalt from 0.1 to 3 per cent.

2. A tool of the character described, consisting of a steel alloy containing copper, zirconium and cobalt in proportions of from 0.1 to 3 per cent, along with other substances such as nickel, chrome and tungsten 75 in the usual percentages which tend to increase its resistive powers.

In testimony whereof I have affixed my signature.

ERNST G. HONES.